# EUROPEAN PATENT SPECIFICATION

(11) **EP 1 881 507 B1**
(45) Date of publication and mention of the grant of the patent: **02.09.2009**
(21) Application number: 06014269.2
(22) Date of filing: 10.07.2006
(51) Int. Cl.: H01B 3/44, H01B 7/02, H01B 9/00

(54) **Cable layer on polypropylene basis with high electrical breakdown strength**
Kabelschicht auf der Basis von Polypropylen mit hoher elektrischer Ausfall-Spannungsfestigkeit
Cables en nappé a base de polypropylene presentant une meilleure résistance au claquage diélectrique

(43) Date of publication of application: 23.01.2008
(62) Divisional of application: 07001886.6
(73) Proprietor: Borealis Technology Oy, 06101 Porvoo (FI)
(72) Inventor: Loyens, Wendy, 444 53 Stenungsund (SE); Eklind, Hans, 444 45 Stenungsund (SE); Stadlbauer, Manfred, 4040 Linz (AT); Ernst, Eberhard, 4210 Unterweitersdorf (AT); Huhtanen, Lauri, 07940 Loviisa (FI)
(74) Representative: Lux, Berthold

(56) References cited:
- EP-A- 1 429 346
- EP-A1- 0 885 918
- EP-A1- 0 893 802
- EP-A2- 0 384 431
- EP-A2- 0 674 325
- EP-A2- 0 690 458

## Description

The present invention relates to a cable layer on polypropylene basis with high electrical breakdown strength. Furthermore, it relates to a process for the preparation of such a cable layer and to cables comprising at least one of these layers.

Today, polyethylene is used as the material of choice for the insulation and semiconductive layers in power cables due to the ease of processing and the beneficial electrical properties. In order to assure good operating properties at the required operating temperature, there is a need to crosslink polyethylene either by peroxides or silanes. However, as a result of crosslinking, there are less recycling options and there is limited processing speed due to dependency on the crosslinking speed. As these are significant drawbacks, replacement of crosslinked polyethylene for cable layers is of great interest.

A potential candidate for replacement is polypropylene. However, polypropylene prepared by the use of Ziegler-Natta catalysts usually has low electrical breakdown strength values.

Of course, any replacement material to be chosen should still have good mechanical and thermal properties enabling failure-free long-run operation of the power cable. Furthermore, any improvement in processability should not be achieved on the expense of mechanical properties and any improved balance of processability and mechanical properties should still result in a material of high electrical breakdown strength.

EP 0893802 A1 discloses cable coating layers comprising a mixture of a crystalline propylene homopolymer or copolymer and a copolymer of ethylene with at least one alpha-olefin. For the preparation of both polymeric components, a metallocene catalyst can be used. Electrical breakdown strength properties are not discussed.

Considering the problems outlined above, it is an object of the present invention to provide a cable layer of high electrical breakdown strength and having a good balance between processability and mechanical properties.

The present invention is based on the finding that an increase in electrical breakdown strength in combination with good processability and mechanical properties can be accomplished with polypropylene by choosing a specific degree of branching of the polymeric backbone. In particular, the polypropylene of the present invention shows a specific degree of short-chain branching. As the branching degree to some extent affects the crystalline structure of the polypropylene, in particular the lamellae thickness distribution, an alternative definition of the polymer of the present invention can be made via its crystallization behaviour.

In the present invention, a cable layer is provided comprising polypropylene, according to claim 1.

It has been recognized that higher electrical breakdown strength is achievable in case the polymer comprises rather high amounts of thin lamellae. Thus the acceptance of the layer as a cable layer is independent from the amount of impurities present in the polypropylene but from its crystalline properties. The stepwise isothermal segregation technique (SIST) provides a possibility to determine the lamellar thickness distribution. Rather high amounts of polymer fractions crystallizing at lower temperatures indicate a rather high amount of thin lamellae. Thus in the present invention, a cable layer is provide comprising polypropylene, wherein said layer and/or the polypropylene comprise(s) a crystalline fraction crystallizing in the temperature range of 200 to 105 °C determined by stepwise isothermal segregation technique (SIST), wherein said crystalline fraction comprises a part which during subsequent melting at a melting rate of 10 °C/min melts at or below the temperature T = Tm-3°C, wherein Tm is the melting temperature, and said part represents at least 45 wt-%, more preferably at least 50 wt-% and yet more preferably at least 55 wt-%, of said crystalline fraction.

Preferably, the cable layer and/or the polypropylene of the layer comprise(s) a crystalline fraction crystallizing in the temperature range of 200 to 105 °C determined by stepwise isothermal segregation technique (SIST), wherein said crystalline fraction comprises a part which during subsequent-melting at a melting rate of 10 °C/min melts at or below 140°C and said part represents at least 15 wt.-%, still more preferably at least 20 wt.-% and yet more preferably at least 25 wt.-% of said crystalline fraction.

The cable layer and/or the polypropylene component of the layer according to the present invention is/are characterized in particular by extensional melt flow properties. The extensional flow, or deformation that involves the stretching of a viscous material, is the dominant type of deformation in converging and squeezing flows that occur in typical polymer processing operations. Extensional melt flow measurements are particularly useful in polymer characterization because they are very sensitive to the molecular structure of the polymeric system being tested. When the true strain rate of extension, also referred to as the Hencky strain rate, is constant, simple extension is said to be a "strong flow" in the sense that it can generate a much higher degree of molecular orientation and stretching than flows in simple shear. As a consequence, extensional flows are very sensitive to crystallinity and macro-structural effects, such as short-chain branching, and as such can be far more descriptive with regard to polymer characterization than other types of bulk rheological measurement which apply shear flow.

Accordingly the cable layer and/or the polypropylene component of the cable layer preferably has/have a strain hardening index *(SHI@1s⁻¹)* of at least 0.15, more preferred of at least 0.20, yet more preferred the strain hardening index *(SHI@1s⁻¹)* is in the range of 0.15 to 0.30. In a further embodiment it is preferred that the cable layer and/or the polypropylene component of the cable layer has/have a strain hardening index (*SHI@1s⁻¹*) in the range of 0.20 to 0.30. The strain hardening index (SHI@1s⁻¹) is measured at a deformation rate dε/dt of 1.00 s⁻¹ at a temperature of 180°C, wherein the strain hardening index (SHI) is defined as the slope of the logarithm to the basis 10 of the tensile stress growth function (Ig(η_{E}⁺)) as a function of the logarithm to the basis 10 of the Hencky strain (I(ε)) in the range of Hencky strains between 1 and 3.

The strain hardening index is a measure for the strain hardening behavior of the polypropylene melt. Moreover values of the strain hardening index (*SHI@1s⁻¹*) of more than 0.10 indicate a non-linear polymer, i.e. a short-chain branched polymer. In the present invention, the strain hardening index (*SHI@1s⁻¹*) is measured by a deformation rate *d*ε/*dt* of 1.00 s⁻¹ at a temperature of 180 °C for determining the strain hardening behavior, wherein the strain hardening index (*SHI@1s⁻¹*) is defined as the slope of the tensile stress growth function *η_{E}⁺* as a function of the Hencky strain ε on a logarithmic scale between 1.00 and 3.00 (see figure 1). Thereby the Hencky strain ε is defined by the formula ε = ε̇*_{H}·t,* wherein
the Hencky strain rate ε̇*_{H}* is defined by the formula ${\dot{ε}}_{H} = \frac{2 ⋅ Ω ⋅ R}{{L}_{0}}$ with
"L₀" is the fixed, unsupported length of the specimen sample being stretched which is equal to the centerline distance between the master and slave drums
"R" is the radius of the equi-dimensional windup drums, and
"Ω" is a constant drive shaft rotation rate.

In turn the tensile stress growth function η*_{E}*⁺ is defined by the formula ${η}_{E}^{+} \left(ε\right) = \frac{F \left(ε\right)}{{\dot{ε}}_{H} ⋅ A \left(ε\right)}$ with $T \left(ε\right) = 2 ⋅ R ⋅ F \left(ε\right)$ and $A \left(ε\right) = {A}_{0} ⋅ {\left(\frac{{d}_{S}}{{d}_{M}}\right)}^{2 / 3} ⋅ exp \left(-ε\right)$ wherein
the Hencky strain rate ε̇*_{H}* is defined as for the Hencky strain ε
"F" is the tangential stretching force
"R" is the radius of the equi-dimensional windup drums
"T" is the measured torque signal, related to the tangential stretching force "F"
"A" is the instantaneous cross-sectional area of a stretched molten specimen
"*A*₀" is the cross-sectional area of the specimen in the solid state (i.e. prior to melting),
"dₛ" is the solid state density and
"d_{M}" the melt density of the polymer.

With the present invention, it is possible to provide a cable layer having high electrical breakdown strength values which are not dependent on the amount of impurities such as aluminium and/or boron residues resulting from the catalyst. Thus, even when the amount of these residues is increasing, a high electrical breakdown strength can be maintained. On the other hand, with the present invention, it is possible to obtain a cable layer having a very low amount of impurities.

Preferably, the cable layer and/or the polypropylene has/have an aluminium residue content of less than 15 ppm, more preferably less than 10 ppm, and/or a boron residue content of less than 15 ppm, more preferably less than 10 ppm.

Preferably, the cable layer and/or the polypropylene of said cable layer has/have xylene solubles below 1.5 wt%, more preferably below 1.0 wt%. A preferred lower limit of xylene solubles is 0.5 wt%. In a preferred embodiment, the cable layer and/or the polypropylene of said cable layer has/have xylene solubles in the range of 0.5 wt% to 1.5 wt%. Xylene solubles are the part of the polymer soluble in cold xylene determined by dissolution in boiling xylene and letting the insoluble part crystallize from the cooling solution (for the method see below in the experimental part). The xylene solubles fraction contains polymer chains of low stereoregularity and is an indication for the amount of non-crystalline areas.

In addition, it is preferred that the crystalline fraction which crystallizes between 200 to 105 °C determined by stepwise isothermal segregation technique (SIST) is at least 90 wt.-% of the total cable layer and/or the total polypropylene, more preferably at least 95 wt.-% of the total layer and/or the total polypropylene and yet more preferably 98 wt.-% of the total layer and/or the total polypropylene.

Preferably, the polypropylene component of the cable layer of the present invention has a tensile modulus of at least 700 MPa measured according to ISO 527-3 at a cross head speed of 1 mm/min.

Another physical parameter which is sensitive to crystallinity and macro-structural effects is the so-called multi-branching index (*MBI*), as will be explained below in further detail.

Similarly to the measurement of *SHI@1s⁻¹,* a strain hardening index (*SHI*) can be determined at different strain rates. A strain hardening index (*SHI*) is defined as the slope of the logarithm to the basis 10 of the tensile stress growth function *η_{E}*⁺, Ig(η*_{E}*⁺), as function of the logarithm to the basis 10 of the Hencky strain ε, Ig(ε), between Hencky strains 1.00 and 3.00 at a temperature of 180 °C, wherein a *SHI@0.1 s⁻¹* is determined with a deformation rate ε̇*_{H}* of 0.10 s⁻¹, a *SHI@0.3 s⁻¹* is determined with a deformation rate ε̇*_{H}* of 0.30 s⁻¹, a *SHI@3.0 s⁻¹* is determined with a deformation rate ε̇*_{H}* of 3.00 s⁻¹, a *SHI@10.0 s⁻¹* is determined with a deformation rate ε̇*_{H}* of 10.0 s⁻¹. In comparing the strain hardening index *(SHI)* at those five strain rates ε̇*_{H}* of 0.10, 0.30, 1.00, 3.00 and 10.00 s⁻¹, the slope of the strain hardening index *(SHI)* as function of the logarithm on the basis 10 of ε̇*_{H}, Ig(*ε̇*_{H})*, is a characteristic measure for short-chain-branching. Therefore, a multi-branching index *(MBI)* is defined as the slope of the strain hardening index (*SHI*) as a function of I*g*(ε̇*_{H}*), i.e. the slope of a linear fitting curve of the strain hardening index (*SHI*) versus I*g*(ε̇*_{H}*) applying the least square method, preferably the strain hardening index *(SHI)* is defined at deformation rates ε̇*_{H}* between 0.05 s⁻¹ and 20.00 s⁻¹, more preferably between 0.10 s⁻¹ and 10.00 s⁻¹, still more preferably at the deformations rates 0.10, 0.30, 1.00, 3.00 and 10.00 s⁻¹.Yet more preferably the *SHI*-values determined by the deformations rates 0.10, 0.30, 1.00, 3.00 and 10.00 s⁻¹ are used for the linear fit according to the least square method when establishing the multi-branching index (*MBI*).

Preferably, the polypropylene component of the cable layer has a multi-branching index (*MBI*) of at least 0.10, more preferably at least 0.15, yet more preferably the multi-branching index (*MBI*) is in the range of 0.10 to 0.30. In a preferred embodiment the polypropylene has a multi-branching index (*MBI*) in the range of 0.15 to 0.30.

The polypropylene component of the cable layer of the present invention is characterized by the fact that the strain hardening index *(SHI)* increases to some extent with the deformation rate ε̇*_{H}* (i.e. short-chain branched polypropylenes), i.e. a phenomenon which is not observed in linear polypropylenes. Single branched polymer types (so called Y polymers having a backbone with a single long side-chain and an architecture which resembles a "Y") or H-branched polymer types (two polymer chains coupled with a bridging group and a architecture which resemble an "H") as well as linear polymers do not show such a relationship, i.e. the strain hardening index (*SHI*) is not influenced by the deformation rate (see Figure 2). Accordingly, the strain hardening index *(SHI)* of known polymers, in particular known polypropylenes, does not increase with increase of the deformation rate (*d*ε/*dt*). Industrial conversion processes which imply elongational flow operate at very fast extension rates. Hence the advantage of a material which shows more pronounced strain hardening (measured by the strain hardening index *SHI*) at high strain rates becomes obvious. The faster the material is stretched, the higher the strain hardening index and hence the more stable the material will be in conversion.

When measured on the cable layer, the multi-branching index (*MBI*) is at least 0.10, more preferably of at least 0.15, yet more preferably the multi-branching index (*MBI*) is in the range of 0.10 to 0.30. In a preferred embodiment the layer has a multi-branching index (*MBI*) in the range of 0.15 to 0.30.

Additionally the polypropylene of the cable layer of the present invention has preferably a branching index g' of less than 1.00. Still more preferably the branching index g' is more than 0.7. Thus it is preferred that the branching index g' of the polypropylene is in the range of more than 0.7 to below 1.0. The branching index g' defines the degree of branching and correlates with the amount of branches of a polymer. The branching index g' is defined as g'=[IV]_{br}/[IV]ₗᵢₙ in which g' is the branching index, [IV_{br}] is the intrinsic viscosity of the branched polypropylene and [IV]ₗᵢₙ is the intrinsic viscosity of the linear polypropylene having the same weight average molecular weight (within a range of ±3%) as the branched polypropylene. Thereby, a low g'-value is an indicator for a high branched polymer. In other words, if the g'-value decreases, the branching of the polypropylene increases. Reference is made in this context to B.H. Zimm and W.H. Stockmeyer, J. Chem. Phys. 17,1301 (1949). This document is herewith included by reference.

The intrinsic viscosity needed for determining the branching index g' is measured according to DIN ISO 1628/1, October 1999 (in decalin at 135 °C).

When measured on the cable layer, the branching index g' is preferably in the range of more than 0.7 to below 1.0.

For further information concerning the measuring methods applied to obtain the relevant data for the branching index g', the tensile stress growth function η*_{E}*⁺, the Hencky strain rate ε̇*_{H}*, the Hencky strain ε and the multi-branching index (*MBI*) it is referred to the example section.

The molecular weight distribution (MWD) (also determined herein as polydispersity) is the relation between the numbers of molecules in a polymer and the individual chain length. The molecular weight distribution (MWD) is expressed as the ratio of weight average molecular weight (M_{w}) and number average molecular weight (Mₙ). The number average molecular weight (Mₙ) is an average molecular weight of a polymer expressed as the first moment of a plot of the number of molecules in each molecular weight range against the molecular weight. In effect, this is the total molecular weight of all molecules divided by the number of molecules. In turn, the weight average molecular weight (M_{w}) is the first moment of a plot of the weight of polymer in each molecular weight range against molecular weight.

The number average molecular weight (Mₙ) and the weight average molecular weight (M_{w}) as well as the molecular weight distribution (MWD) are determined by size exclusion chromatography (SEC) using Waters Alliance GPCV 2000 instrument with online viscometer. The oven temperature is 140 °C. Trichlorobenzene is used as a solvent (ISO 16014).

It is preferred that the cable layer of the present invention comprises a polypropylene which has a weight average molecular weight (M_{w}) from 10,000 to 2,000,000 g/mol, more preferably from 20,000 to 1,500,000 g/mol.

The number average molecular weight (Mₙ) of the polypropylene is preferably in the range of 5,000 to 1,000,000 g/mol, more preferably from 10,000 to 750,000 g/mol.

As a broad molecular weight distribution (MWD) improves the processability of the polypropylene the molecular weight distribution (MWD) is preferably up to 20.00, more preferably up to 10.00, still more preferably up to 8.00. However a rather broad molecular weight distribution simulates sagging. Therefore, in an alternative embodiment the molecular weight distribution (MWD) is preferably between 1.00 to 8.00, still more preferably in the range of 1.00 to 4.00, yet more preferably in the range of 1.00 to 3.50.

Furthermore, it is preferred that the polypropylene component of the cable layer of the present invention has a melt flow rate (MFR) given in a specific range. The melt flow rate mainly depends on the average molecular weight. This is due to the fact that long molecules render the material a lower flow tendency than short molecules. An increase in molecular weight means a decrease in the MFR-value. The melt flow rate (MFR) is measured in g/10 min of the polymer discharged through a defined die under specified temperature and pressure conditions and the measure of viscosity of the polymer which, in turn, for each type of polymer is mainly influenced by its molecular weight but also by its degree of branching. The melt flow rate measured under a load of 2.16 kg at 230 °C (ISO 1133) is denoted as MFR₂. Accordingly, it is preferred that in the present invention the cable layer comprises a polypropylene which has an MFR₂ up to 8.00 g/10min, more preferably up to 6.00 g/10min. In another preferred embodiment the polypropylene has MFR₂ up to 4 g/10min. A preferred range for the MFR₂ is 1.00 to 40.00 g/10 min, more preferably in the range of 1.00 to 30.00 g/10min, yet more preferably in the range of 2.00 to 30.00 g/10min.

As cross-linking has a detrimental effect on the extensional flow properties it is preferred that the polypropylene according to this invention is non-cross-linked.

The polypropylene of the cable layer according to this invention shall have a rather high isotacticity measured by meso pentad concentration (also referred herein as pentad concentration), i.e. higher than 91 %, more preferably higher than 93 %, still more preferably higher than 94 % and most preferably higher than 95 %. On the other hand pentad concentration shall be not higher than 99.5 %. The pentad concentration is an indicator for the narrowness in the regularity distribution of the polypropylene and measured by NMR-spectroscopy.

In addition, it is preferred that the cable layer and/or the polypropylene of the said layer has/have a melting temperature Tm of higher than 148 °C, more preferred higher than 150 °C. In a preferred embodiment, melting temperature Tm of the polypropylene component is higher than 148 °C but below 160 °C. The measuring method for the melting temperature Tm is discussed in the example section.

Moreover it is preferred that the cable layer according to this invention has an electrical breakdown strength EB63% measured according to IEC 60243-part 1 (1988) of at least 135.5 kV/mm, more preferably at least 138 kV/mm, even more preferably at least 140 kV/mm. Further details about electrical breakdown strength are provided below in the examples.

In a preferred embodiment the polypropylene as defined above (and further defined below) is preferably unimodal. In another preferred embodiment the polypropylene as defined above (and further defined below) is preferably multimodal, more preferably bimodal.

"Multimodal" or "multimodal distribution" describes a frequency distribution that has several relative maxima (contrary to unimodal having only one maximum). In particular, the expression "modality of a polymer" refers to the form of its molecular weight distribution (MWD) curve, i.e. the appearance of the graph of the polymer weight fraction as a function of its molecular weight. If the polymer is produced in the sequential step process, i.e. by utilizing reactors coupled in series, and using different conditions in each reactor, the different polymer fractions produced in the different reactors each have their own molecular weight distribution which may considerably differ from one another. The molecular weight distribution curve of the resulting final polymer can be seen at a super-imposing of the molecular weight distribution curves of the polymer fraction which will, accordingly, show a more distinct maxima, or at least be distinctively broadened compared with the curves for individual fractions.

A polymer showing such molecular weight distribution curve is called bimodal or multimodal, respectively.

In case the polypropylene of the cable layer is not unimodal it is preferably bimodal.

The polypropylene of the cable layer according to this invention can be a homopolymer or a copolymer. In case the polypropylene is unimodal the polypropylene is preferably a polypropylene homopolymer. In turn in case the polypropylene is multimodal, more preferably bimodal, the polypropylene can be a polypropylene homopolymer as well as a polypropylene copolymer. Furthermore, it is preferred that at least one of the fractions of the multimodal polypropylene is a short-chain branched polypropylene, preferably a short-chain branched polypropylene homopolymer, as defined above.

The expression polypropylene homopolymer as used in this invention relates to a polypropylene that consists substantially, i.e. of at least 97 wt%, preferably of at least 99 wt%, and most preferably of at least 99.8 wt% of propylene units. In a preferred embodiment only propylene units in the polypropylene homopolymer are detectable. The comonomer content can be measured with FT infrared spectroscopy. Further details are provided below in the examples.

In case the polypropylene of the layer according to this invention is a multimodal or bimodal polypropylene copolymer, it is preferred that the comonomer is ethylene. However, also other comonomers known in the art are suitable. Preferably, the total amount of comonomer, more preferably ethylene, in the propylene copolymer is up to 30 wt%, more preferably up to 25 wt%.

In a preferred embodiment, the multimodal or bimodal polypropylene copolymer is a polypropylene copolymer comprising a polypropylene homopolymer matrix being a short chain branched polypropylene as defined above and an ethylene-propylene rubber (EPR).

The polypropylene homopolymer matrix can be unimodal or multimodal, i.e. bimodal. However it is preferred that polypropylene homopolymer matrix is unimodal.

Preferably, the ethylene-propylene rubber (EPR) in the total multimodal or bimodal polypropylene copolymer is up to 80 wt%. More preferably the amount of ethylene-propylene rubber (EPR) in the total multimodal or bimodal polypropylene copolymer is in the range of 10 to 70 wt%, still more preferably in the range of 10 to 60 wt%.

In addition, it is preferred that the multimodal or bimodal polypropylene copolymer comprises a polypropylene homopolymer matrix being a short chain branched polypropylene as defined above and an ethylene-propylene rubber (EPR) with an ethylene-content of up to 50 wt%.

In addition, it is preferred that the polypropylene as defined above is produced in the presence of the catalyst as defined below. Furthermore, for the production of the polypropylene as defined above, the process as stated below is preferably used.

The polypropylene of the cable layer according to this invention has been in particular obtained by a new catalyst system. This new catalyst system comprises a symmetric catalyst, whereby the catalyst system has a porosity of less than 1.40 ml/g, more preferably less than 1.30 ml/g and most preferably less than 1.00 ml/g. The porosity has been measured according to DIN 66135 (N₂). In another preferred embodiment the porosity is not detectable when determined with the method applied according to DIN 66135 (N₂).

A symmetric catalyst according to this invention is a metallocene compound having a C₂-symetry. Preferably the C₂-symetric metallocene comprises two identical organic ligands, still more preferably comprises only two organic ligands which are identical, yet more preferably comprises only two organic ligands which are identical and linked via a bridge.

Said symmetric catalyst is preferably a single site catalyst (SSC).

Due to the use of the catalyst system with a very low porosity comprising a symmetric catalyst the manufacture of the above defined short-chain branched polypropylene is possible.

Furthermore it is preferred, that the catalyst system has a surface area of lower than 25 m²/g, yet more preferred lower than 20 m²/g, still more preferred lower than 15 m²/g, yet still lower than 10 m²/g and most preferred lower than 5 m²/g. The surface area according to this invention is measured according to ISO 9277 (N₂).

It is in particular preferred that the catalytic system according to this invention comprises a symmetric catalyst, i.e. a catalyst as defined above and in further detail below, and has porosity not detectable when applying the method according to DIN 66135 (N₂) and has a surface area measured according to ISO 9277 (N₂) of less than 5 m²/g.

Preferably the symmetric catalyst compound, i.e. the C₂-symetric metallocene, has the formula (I):

(Cp)₂R₁MX₂ (I)

wherein
M is Zr, Hf or Ti, more preferably Zr, and
X is independently a monovalent anionic ligand, such as σ-ligand
R is a bridging group linking the two Cp ligands
Cp is an organic ligand selected from the group consisting of unsubstituted cyclopenadienyl, unsubstituted indenyl, unsubstituted tetrahydroindenyl, unsubstituted fluorenyl, substituted cyclopenadienyl, substituted indenyl, substituted tetrahydroindenyl, and substituted fluorenyl,
with the proviso that both Cp-ligands are selected from the above stated group and both Cp-ligands are chemically the same, i.e. are identical.

The term "σ-ligand" is understood in the whole description in a known manner, i.e. a group bonded to the metal at one or more places via a sigma bond. A preferred monovalent anionic ligand is halogen, in particular chlorine (Cl).

Preferably, the symmetric catalyst is of formula (I) indicated above,
wherein
M is Zr and
each X is Cl.

Preferably both identical Cp-ligands are substituted.

The optional one or more substituent(s) bonded to cyclopenadienyl, indenyl, tetrahydroindenyl, or fluorenyl may be selected from a group including halogen, hydrocarbyl (e.g. C₁-C₂₀-alkyl, C₂-C₂₀-alkenyl, C₂-C₂₀-alkynyl, C₃-C₁₂-cycloalkyl, C₆-C₂₀-aryl or C₇-C₂₀-arylalkyl), C₃-C₁₂-cycloalkyl which contains 1, 2, 3 or 4 heteroatom(s) in the ring moiety, C₆-C₂₀-heteroaryl, C₁-C₂₀-haloalkyl, -SiR"₃, -OSiR"₃, -SR", -PR"₂ and -NR"₂, wherein each R" is independently a hydrogen or hydrocarbyl, e.g. C₁-C₂₀-alkyl, C₂-C₂₀-alkenyl, C₂-C₂₀-alkynyl, C₃-C₁₂-cycloalkyl or C₆-C₂₀-aryl.

More preferably both identical Cp-ligands are indenyl moieties wherein each indenyl moiety bear one or two substituents as defined above. More preferably each of the identical Cp-ligands is an indenyl moiety bearing two substituents as defined above, with the proviso that the substituents are chosen in such are manner that both Cp-ligands are of the same chemical structure, i.e both Cp-ligands have the same substituents bonded to chemically the same indenyl moiety.

Still more preferably both identical Cp's are indenyl moieties wherein the indenyl moieties comprise at least at the five membered ring of the indenyl moiety, more preferably at 2-position, a substituent selected from the group consisting of alkyl, such as C₁-C₆ alkyl, e.g. methyl, ethyl, isopropyl, and trialkyloxysiloxy, wherein each alkyl is independently selected from C₁-C₆ alkyl, such as methyl or ethyl, with proviso that the indenyl moieties of both Cp are of the same chemical structure, i.e both Cp-ligands have the same substituents bonded to chemically the same indenyl moiety.

Still more preferred both identical Cp's are indenyl moieties wherein the indenyl moieties comprise at least at the six membered ring of the indenyl moiety, more preferably at 4-position, a substituent selected from the group consisting of a C₆-C₂₀ aromatic ring moiety, such as phenyl or naphthyl, preferably phenyl, which is optionally substituted with one or more substitutents, such as C₁-C₆ alkyl, and a heteroaromatic ring moiety, with proviso that the indenyl moieties of both Cp are of the same chemical structure, i.e both Cp-ligands have the same substituents bonded to chemically the same indenyl moiety.

Yet more preferably both identical Cp are indenyl moieties wherein the indenyl moieties comprise at the five membered ring of the indenyl moiety, more preferably at 2-position, a substituent and at the six membered ring of the indenyl moiety, more preferably at 4-position, a further substituent, wherein the substituent of the five membered ring is selected from the group consisting of alkyl, such as C₁-C₆ alkyl, e.g. methyl, ethyl, isopropyl, and trialkyloxysiloxy and the further substituent of the six membered ring is selected from the group consisting of a C₆-C₂₀ aromatic ring moiety, such as phenyl or naphthyl, preferably phenyl, which is optionally substituted with one or more substituents, such as C₁-C₆ alkyl, and a heteroaromatic ring moiety, with proviso that the indenyl moieties of both Cp's are of the same chemical structure, i.e both Cp-ligands have the same substituents bonded to chemically the same indenyl moiety.

Concerning the moiety "R" it is preferred that "R" has the formula (II)

-Y(R')₂- (II)

wherein
Y is C, Si or Ge, and
R' is C₁ to C₂₀ alkyl, C₆-C₁₂ aryl, or C₇-C₁₂ arylalkyl or trimethylsilyl.

In case both Cp-ligands of the symmetric catalyst as defined above, in particular case of two indenyl moieties, are linked with a bridge member R, the bridge member R is typically placed at 1-position. The bridge member R may contain one or more bridge atoms selected from e.g. C, Si and/or Ge, preferably from C and/or Si. One preferable bridge R is -Si(R')₂-, wherein R' is selected independently from one or more of e.g. trimethylsilyl, C₁-C₁₀ alkyl, C₁-C₂₀ alkyl, such as C₆-C₁₂ aryl, or C₇-C₄₀, such as C₇-C₁₂ arylalkyl, wherein alkyl as such or as part of arylalkyl is preferably C₁-C₆ alkyl, such as ethyl or methyl, preferably methyl, and aryl is preferably phenyl. The bridge -Si(R')₂- is preferably e.g. -Si(C₁-C₆ alkyl)₂-, -Si(phenyl)₂- or -Si(C₁-C₆ alkyl)(phenyl)-, such as -Si(Me)₂-.

In a preferred embodiment the symmetric catalyst, i.e. the C₂-symetric metallocene, is defined by the formula (III)

(Cp)₂R₁ZrCl₂ (III)

wherein
both Cp coordinate to M and are selected from the group consisting of unsubstituted cyclopenadienyl, unsubstituted indenyl, unsubstituted tetrahydroindenyl, unsubstituted fluorenyl, substituted cyclopenadienyl, substituted indenyl, substituted tetrahydroindenyl, and substituted fluorenyl,
with the proviso that both Cp-ligands are chemically the same, i.e. are identical, and
R is a bridging group linking two ligands L,
wherein R is defined by the formula (II)

-Y(R')₂- (II)

wherein
Y is C, Si or Ge, and
R' is C₁ to C₂₀ alkyl, C₆-C₁₂ aryl, or C₇-C₁₂ arylalkyl.

More preferably the symmetric catalyst is defined by the formula (III), wherein both Cp are selected from the group consisting of substituted cyclopenadienyl, substituted indenyl, substituted tetrahydroindenyl, and substituted fluorenyl.

In a preferred embodiment the symmetric catalyst is dimethylsilyl(2-methyl-4-phenyl-indenyl)₂zirkonium dichloride. More preferred said symmetric catalyst is non-silica supported.

The above described symmetric catalyst components are prepared according to the methods described in WO 01/48034.

It is in particular preferred that the symmetric catalyst is obtainable by the emulsion solidification technology as described in WO 03/051934. This document is herewith included in its entirety by reference. Hence the symmetric catalyst is preferably in the form of solid catalyst particles, obtainable by a process comprising the steps of
a) preparing a solution of one or more symmetric catalyst components;
b) dispersing said solution in a solvent immiscible therewith to form an emulsion in which said one or more catalyst components are present in the droplets of the dispersed phase,
c) solidifying said dispersed phase to convert said droplets to solid particles and optionally recovering said particles to obtain said catalyst.

Preferably a solvent, more preferably an organic solvent, is used to form said solution. Still more preferably the organic solvent is selected from the group consisting of a linear alkane, cyclic alkane, linear alkene, cyclic alkene, aromatic hydrocarbon and halogen-containing hydrocarbon.

Moreover the immiscible solvent forming the continuous phase is an inert solvent, more preferably the immiscible solvent comprises a fluorinated organic solvent and/or a functionalized derivative thereof, still more preferably the immiscible solvent comprises a semi-, highly- or perfluorinated hydrocarbon and/or a functionalized derivative thereof. It is in particular preferred, that said immiscible solvent comprises a perfluorohydrocarbon or a functionalized derivative thereof, preferably C₃-C₃₀ perfluoroalkanes, -alkenes or -cycloalkanes, more preferred C₄-C₁₀ perfluoroalkanes, -alkenes or -cycloalkanes, particularly preferred perfluorohexane, perfluoroheptane, perfluorooctane or perfluoro (methylcyclohexane) or a mixture thereof.

Furthermore it is preferred that the emulsion comprising said continuous phase and said dispersed phase is a bi-or multiphasic system as known in the art. An emulsifier may be used for forming the emulsion. After the formation of the emulsion system, said catalyst is formed in situ from catalyst components in said solution.

In principle, the emulsifying agent may be any suitable agent which contributes to the formation and/or stabilization of the emulsion and which does not have any adverse effect on the catalytic activity of the catalyst. The emulsifying agent may e.g. be a surfactant based on hydrocarbons optionally interrupted with (a) heteroatom(s), preferably halogenated hydrocarbons optionally having a functional group, preferably semi-, highly- or perfluorinated hydrocarbons as known in the art. Alternatively, the emulsifying agent may be prepared during the emulsion preparation, e.g. by reacting a surfactant precursor with a compound of the catalyst solution. Said surfactant precursor may be a halogenated hydrocarbon with at least one functional group, e.g. a highly fluorinated C₁ to C₃₀ alcohol, which reacts e.g. with a cocatalyst component, such as aluminoxane.

In principle any solidification method can be used for forming the solid particles from the dispersed droplets. According to one preferable embodiment the solidification is effected by a temperature change treatment. Hence the emulsion subjected to gradual temperature change of up to 10 °C/min, preferably 0.5 to 6 °C/min and more preferably 1 to 5 °C/min. Even more preferred the emulsion is subjected to a temperature change of more than 40 °C, preferably more than 50 °C within less than 10 seconds, preferably less than 6 seconds.

The recovered particles have preferably an average size range of 5 to 200 µm, more preferably 10 to 100 µm.

Moreover, the form of solidified particles have preferably a spherical shape, a predetermined particles size distribution and a surface area as mentioned above of preferably less than 25 m²/g, still more preferably less than 20 m²/g, yet more preferably less than 15 m²/g, yet still more preferably less than 10 m²/g and most preferably less than 5 m²/g, wherein said particles are obtained by the process as described above.

For further details, embodiments and examples of the continuous and dispersed phase system, emulsion formation method, emulsifying agent and solidification methods reference is made e.g. to the above cited international patent application WO 03/051934.

The above described symmetric catalyst components are prepared according to the methods described in WO 01/48034.

As mentioned above the catalyst system may further comprise an activator as a cocatalyst, as described in WO 03/051934, which is enclosed herein with reference.

Preferred as cocatalysts for metallocenes and non-metallocenes, if desired, are the aluminoxanes, in particular the C₁-C₁₀-alkylaluminoxanes, most particularly methylaluminoxane (MAO). Such aluminoxanes can be used as the sole cocatalyst or together with other cocatalyst(s). Thus besides or in addition to aluminoxanes, other cation complex forming catalysts activators can be used. Said activators are commercially available or can be prepared according to the prior art literature.

Further aluminoxane cocatalysts are described i.a. in WO 94/28034 which is incorporated herein by reference. These are linear or cyclic oligomers of having up to 40, preferably 3 to 20, -(AI(R"')O)- repeat units (wherein R"' is hydrogen, C₁-C₁₀-alkyl (preferably methyl) or C₆-C₁₈-aryl or mixtures thereof).

The use and amounts of such activators are within the skills of an expert in the field. As an example, with the boron activators, 5:1 to 1:5, preferably 2:1 to 1:2, such as 1:1, ratio of the transition metal to boron activator may be used. In case of preferred aluminoxanes, such as methylaluminumoxane (MAO), the amount of Al, provided by aluminoxane, can be chosen to provide a molar ratio of Al:transition metal e.g. in the range of 1 to 10 000, suitably 5 to 8000, preferably 10 to 7000, e.g. 100 to 4000, such as 1000 to 3000. Typically in case of solid (heterogeneous) catalyst the ratio is preferably below 500.

The quantity of cocatalyst to be employed in the catalyst of the invention is thus variable, and depends on the conditions and the particular transition metal compound chosen in a manner well known to a person skilled in the art.

Any additional components to be contained in the solution comprising the organotransition compound may be added to said solution before or, alternatively, after the dispersing step.

Furthermore, the present invention is related to the use of the above-defined catalyst system for the production of a polypropylene according to this invention.

In addition, the present invention is related to the process for producing the inventive cable layer comprising the polypropylene, whereby the catalyst system as defined above is employed. Furthermore it is preferred that the process temperature is higher than 60 °C. Preferably, the process is a multi-stage process to obtain multimodal polypropylene as defined above.

Multistage processes include also bulk/gas phase reactors known as multizone gas phase reactors for producing multimodal propylene polymer.

A preferred multistage process is a "loop-gas phase"-process, such as developed by Borealis A/S, Denmark (known as BORSTAR® technology) described e.g. in patent literature, such as in EP 0 887 379 or in WO 92/12182.

Multimodal polymers can be produced according to several processes which are described, e.g. in WO 92/12182, EP 0 887 379 and WO 97/22633.

A multimodal polypropylene according to this invention is produced preferably in a multi-stage process in a multi-stage reaction sequence as described in WO 92/12182. The content of this document is included herein by reference.

It has previously been known to produce multimodal, in particular bimodal, polypropylene in two or more reactors connected in series, i.e. in different steps (a) and (b).

According to the present invention, the main polymerization stages are preferably carried out as a combination of a bulk polymerization/gas phase polymerization.

The bulk polymerizations are preferably performed in a so-called loop reactor.

In order to produce the multimodal polypropylene according to this invention, a flexible mode is preferred. For this reason, it is preferred that the composition be produced in two main polymerization stages in combination of loop reactor/gas phase reactor.

Optionally, and preferably, the process may also comprise a prepolymerization step in a manner known in the field and which may precede the polymerization step (a).

If desired, a further elastomeric comonomer component, so called ethylene-propylene rubber (EPR) component as in this invention, may be incorporated into the obtained polypropylene homopolymer matrix to form a propylene copolymer as defined above. The ethylene-propylene rubber (EPR) component may preferably be produced after the gas phase polymerization step (b) in a subsequent second or further gas phase polymerizations using one or more gas phase reactors.

The process is preferably a continuous process.

Preferably, in the process for producing the propylene polymer as defined above the conditions for the bulk reactor of step (a) may be as follows:
- the temperature is within the range of 40 °C to 110 °C, preferably between 60 °C and 100 °C, 70 to 90 °C,
- the pressure is within the range of 20 bar to 80 bar, preferably between 30 bar to 60 bar,
- hydrogen can be added for controlling the molar mass in a manner known per se.

Subsequently, the reaction mixture from the bulk (bulk) reactor (step a) is transferred to the gas phase reactor, i.e. to step (b), whereby the conditions in step (b) are preferably as follows:
- the temperature is within the range of 50 °C to 130 °C, preferably between 60 °C and 100 °C,
- the pressure is within the range of 5 bar to 50 bar, preferably between 15 bar to 35 bar,
- hydrogen can be added for controlling the molar mass in a manner known per se.

The residence time can vary in both reactor zones. In one embodiment of the process for producing the propylene polymer the residence time in bulk reactor, e.g. loop is in the range 0.5 to 5 hours, e.g. 0.5 to 2 hours and the residence time in gas phase reactor will generally be 1 to 8 hours.

If desired, the polymerization may be effected in a known manner under supercritical conditions in the bulk, preferably loop reactor, and/or as a condensed mode in the gas phase reactor.

The process of the invention or any embodiments thereof above enable highly feasible means for producing and further tailoring the propylene polymer composition within the invention, e.g. the properties of the polymer composition can be adjusted or controlled in a known manner e.g. with one or more of the following process parameters: temperature, hydrogen feed, comonomer feed, propylene feed e.g. in the gas phase reactor, catalyst, the type and amount of an external donor (if used), split between components.

The above process enables very feasible means for obtaining the reactor-made polypropylene as defined above.

The cable layer of the present invention can be an insulation layer or a semiconductive layer. In case it is a semiconductive layer, it preferably comprises carbon black.

The present invention also provides a cable, preferably a power cable, comprising a conductor and one or more coating layers, wherein at least one of the coating layers is a cable layer as defined above.

The cable of the present invention can be prepared by processes known to the skilled person, e.g. by extrusion coating of the conductor.

The present invention will now be described in further detail by the examples provided below.

### Examples

### 1. Definitions/Measuring methods

The following definitions of terms and determination methods apply for the above general description of the invention as well as to the below examples unless otherwise defined.

### A. Pentad concentration

For the meso pentad concentration analysis (also referred herein as pentad concentration analysis), the assignment analysis is undertaken according to T Hayashi, Pentad concentration, R. Chujo and T. Asakura, Polymer 29 138-43 (1988) and Chujo R, et al., Polymer 35 339 (1994)

### B. Multi-branching Index

### 1. Acquiring the experimental data

Polymer is melted at T=180 °C and stretched with the SER Universal Testing Platform as described below at deformation rates of dε/dt=0.1 0.3 1.0 3.0 and 10 s⁻¹ in subsequent experiments. The method to acquire the raw data is described in Sentmanat et al., J. Rheol. 2005, Measuring the Transient Elongational Rheology of Polyethylene Melts Using the SER Universal Testing Platform.

### Experimental Setup

A Paar Physica MCR300, equipped with a TC30 temperature control unit and an oven CTT600 (convection and radiation heating) and a SERVP01-025 extensional device with temperature sensor and a software RHEOPLUS/32 v2.66 is used.

### Sample Preparation

Stabilized Pellets are compression moulded at 220°C (gel time 3min, pressure time 3 min, total moulding time 3+3=6min) in a mould at a pressure sufficient to avoid bubbles in the specimen, cooled to room temperature. From such prepared plate of 0.7mm thickness, stripes of a width of 10mm and a length of 18mm are cut.

### Check of the SER Device

Because of the low forces acting on samples stretched to thin thicknesses, any essential friction of the device would deteriorate the precision of the results and has to be avoided.

In order to make sure that the friction of the device less than a threshold of 5x10-3 mNm (Milli-Newtonmeter) which is required for precise and correct measurements, following check procedure is performed prior to each measurement:
- The device is set to test temperature (180°C) for minimum 20minutes without sample in presence of the clamps
- A standard test with 0.3s-1 is performed with the device on test temperature (180°C)
- The torque (measured in mNm) is recorded and plotted against time
- The torque must not exceed a value of 5x10-3 mNm to make sure that the friction of the device is in an acceptably low range

### Conducting the experiment

The device is heated for min. 20min to the test temperature (180°C measured with the thermocouple attached to the SER device) with clamps but without sample. Subsequently, the sample (0.7x10x18mm), prepared as described above, is clamped into the hot device. The sample is allowed to melt for 2 minutes +/- 20 seconds before the experiment is started.

During the stretching experiment under inert atmosphere (nitrogen) at constant Hencky strain rate, the torque is recorded as function of time at isothermal conditions (measured and controlled with the thermocouple attached to the SER device).

After stretching, the device is opened and the stretched film (which is winded on the drums) is inspected. Homogenous extension is required. It can be judged visually from the shape of the stretched film on the drums if the sample stretching has been homogenous or not. The tape must me wound up symmetrically on both drums, but also symmetrically in the upper and lower half of the specimen.

If symmetrical stretching is confirmed hereby, the transient elongational viscosity calculates from the recorded torque as outlined below.

### 2. Evaluation

For each of the different strain rates dε/dt applied, the resulting tensile stress growth function η_{E}⁺ (dε/dt, t) is plotted against the total Hencky strain ε to determine the strain hardening behaviour of the melt, see Figure 1.

In the range of Hencky strains between 1.0 and 3.0, the tensile stress growth function η_{E}⁺ can be well fitted with a function ${η}_{E}^{+} \left(\dot{ε}⁢ε\right) = {c}_{1} ⋅ {ε}^{{c}_{2}}$
where c₁ and c₂ are fitting variables. Such derived c₂ is a measure for the strain hardening behavior of the melt and called Strain Hardening Index SHI.

Dependent on the polymer architecture, SHI can
- be independent of the strain rate (linear materials, Y- or H-structures)
- increase with strain rate (short chain-, hyper- or multi-branched structures).

This is illustrated in Figure 2.

For polyethylene, linear (HDPE), short-chain branched (LLDPE) and hyperbranched structures (LDPE) are well known and hence they are used to illustrate the structural analytics based on the results on extensional viscosity. They are compared with a polypropylene with Y and H-structures with regard to their change of the strain-hardening behavior as function of strain rate, see Figure 2 and Table 1.

To illustrate the determination of *SHI* at different strain rates as well as the multi-branching index (*MBI*) four polymers of known chain architecture are examined with the analytical procedure described above.

The first polymer is a H- and Y-shaped polypropylene homopolymer made according to EP 879 830 ("A"). It has a MFR230/2.16 of 2.0g/10min, a tensile modulus of 1950MPa and a branching index g' of 0.7.

The second polymer is a commercial hyperbranched LDPE, Borealis "B", made in a high pressure process known in the art. It has a MFR190/2.16 of 4.5 and a density of 923kg/m³.

The third polymer is a short chain branched LLDPE, Borealis "C", made in a low pressure process known in the art. It has a MFR190/2.16 of 1.2 and a density of 919kg/m³.

The fourth polymer is a linear HDPE, Borealis "D", made in a low pressure process known in the art. It has a MFR190/2.16 of 4.0 and a density of 954kg/m³.

The four materials of known chain architecture are investigated by means of measurement of the transient elongational viscosity at 180°C at strain rates of 0.10, 0.30, 1.0, 3.0 and 10s⁻¹. Obtained data (transient elongational viscosity versus Hencky strain) is fitted with a function ${η}_{E}^{+} = {c}_{1} * {ε}^{{c}_{2}}$

for each of the mentioned strain rates. The parameters c1 and c2 are found through plotting the logarithm of the transient elongational viscosity against the logarithm of the Hencky strain and performing a linear fit of this data applying the least square method. The parameter c1 calculates from the intercept of the linear fit of the data *Ig*(*η_{E}⁺*) versus *Ig*(ε) from ${c}_{1} = {10}^{Intercept}$ and C₂ is the strain hardening index *(SHI)* at the particular strain rate.

This procedure is done for all five strain rates and hence, SHI@0.1s⁻¹, *SHI@0.3s⁻¹, SHI@1.0s⁻¹, SHI@3.0s⁻¹, SHI@10s⁻¹* are determined, see Figure 1.

| **dε/dt** | **Ig (dε/dt)** | **Property** | **Y and H branched** | **multibranched** | **short-chain branched** | **linear** |
|---|---|---|---|---|---|---|
| | | | **A** | **B** | **C** | **D** |
| 0,1 | -1,0 | SHI@0.1s⁻¹ | 2,05 | - | 0,03 | 0,03 |
| 0,3 | -0,5 | SHI@0.3s⁻¹ | - | 1,36 | 0,08 | 0,03 |
| 1 | 0,0 | SHI@1.0s⁻¹ | 2,19 | 1,65 | 0,12 | 0,11 |
| 3 | 0,5 | SHI@3.0s⁻¹ | - | 1,82 | 0,18 | 0,01 |
| 10 | 1,0 | SHI@10s⁻¹ | 2,14 | 2,06 | - | - |

From the strain hardening behaviour measured by the values of the *SHI@1s⁻¹* one can already clearly distinguish between two groups of polymers: Linear and short-chain branched have a *SHI@1s⁻¹* significantly smaller than 0.30. In contrast, the Y and H-branched as well as hyperbranched materials have a *SHI@1s⁻¹* significantly larger than 0.30.

In comparing the strain hardening index at those five strain rates ε̇*_{H}* of 0.10, 0.30, 1.0, 3.0 and 10s⁻¹, the slope of *SHI* as function of the logarithm of ε̇*_{H}*, *Ig(*ε̇*_{H}) is a characteristic measure for multi* -branching. Therefore, a multi-branching index (*MBI*) is calculated from the slope of a linear fitting curve of *SHI* versus Ig(ε̇*_{H}*): $SHI \left({\dot{ε}}_{H}\right) = c ⁢ 3 + MBI * Ig \left({\dot{ε}}_{H}\right)$

The parameters c3 and *MBI* are found through plotting the SHI against the logarithm of the Hencky strain rate Ig(ε̇*_{H}*) and performing a linear fit of this data applying the least square method. Please confer to Figure 2.

| **Property** | **Y and H branched** | **multibranched** | **short-chain branched** | **linear** |
|---|---|---|---|---|
| | **A** | **B** | **C** | **D** |
| MBI | 0,04 | 0,45 | 0,10 | 0,01 |

The multi-branching index *MBI* allows now to distinguish between Y or H-branched polymers which show a *MBI* smaller than 0.05 and hyperbranched polymers which show a *MBI* larger than 0.15. Further, it allows to distinguish between short-chain branched polymers with *MBI* larger than 0.10 and linear materials which have a *MBI* smaller than 0.10.

Combining both, strain hardening index and multi-branching index, the chain architecture can be assessed as indicated in Table 3:

**Table 3: Strain Hardening Index (SHI) and Multi-branching Index (MBI) for various chain architectures**

| **Property** | **Y and H branched** | **Multi- branched** | **short-chain branched** | **linear** |
|---|---|---|---|---|
| SHI@1.0s⁻¹ | >0.30 | >0.30 | ≤0.30 | ≤0.30 |
| MBI | ≤0.10 | >0.10 | >0.10 | ≤0.10 |

### C. Elementary Analysis

The below described elementary analysis is used for determining the content of elementary residues which are mainly originating from the catalyst, especially the Al-, B-, and Si-residues in the polymer. Said Al-, B- and Si-residues can be in any form, e.g. in elementary or ionic form, which can be recovered and detected from polypropylene using the below described ICP-method. The method can also be used for determining the Ti-content of the polymer. It is understood that also other known methods can be used which would result in similar results.

### ICP-Spectrometry (Inductively Coupled Plasma Emission)

**ICP-instrument:** The instrument for determination of Al-, B- nad Si-content is ICP Optima 2000 DV, PSN 620785 (supplier Perkin Elmer Instruments, Belgium) with software of the instrument.

Detection limits are 0.10 ppm (AI), 0.10 ppm (B), 0.10 ppm (Si).

The polymer sample was first ashed in a known manner, then dissolved in an appropriate acidic solvent. The dilutions of the standards for the calibration curve are dissolved in the same solvent as the sample and the concentrations chosen so that the concentration of the sample would fall within the standard calibration curve.

ppm: means parts per million by weight

**Ash content:** Ash content is measured according to ISO 3451-1 (1997) standard.

### Calculated ash, Al- Si- and B-content:

The ash and the above listed elements, Al and/or Si and/or B can also be calculated form a polypropylene based on the polymerization activity of the catalyst as exemplified in the examples. These values would give the upper limit of the presence of said residues originating form the catalyst.

Thus the estimate catalyst residue is based on catalyst composition and polymerization productivity, catalyst residues in the polymer can be estimated according to: $Total catalyst residues \left[ppm\right] = 1 / productivity \left[{kg}_{pp}/{g}_{catalyst}\right] \times 100$ $Al residues \left[ppm\right] = {w}_{A ⁢ 1 , catalyst} \left[%\right] \times total catalyst residues \left[ppm\right] / 100$ $Zr residues \left[ppm\right] = {w}_{Zr , catalyst} \left[%\right] \times total catalyst residues \left[ppm\right] / 100$ (Similar calculations apply also for B, Cl and Si residues)

**Chlorine residues content:** The content of Cl-residues is measured from samples in the known manner using X-ray fluorescence (XRF) spectrometry. The instrument was X-ray fluorescention Philips PW2400, PSN 620487, (Supplier: Philips, Belgium) software X47. Detection limit for Cl is 1 ppm.

### D. Further Measuring Methods

**Particle size distribution:** Particle size distribution is measured via Coulter Counter LS 200 at room temperature with n-heptane as medium.

### NMR

### NMR-spectroscopy measurements:

The ¹³C-NMR spectra of polypropylenes were recorded on Bruker 400MHz spectrometer at 130 °C from samples dissolved in 1,2,4-trichlorobenzene/benzene-d6 (90/10 w/w). For the pentad analysis the assignment is done according to the methods described in literature: (T. Hayashi, Y. Inoue, R. Chüjö, and T. Asakura, Polymer 29 138-43 (1988).and Chujo R, et al,Polymer 35 339 (1994).

The NMR-measurement was used for determining the mmmm pentad concentration in a manner well known in the art.

**Number average molecular weight (Mₙ), weight average molecular weight (M_{w}) and molecular weight distribution (MWD)** are determined by size exclusion chromatography (SEC) using Waters Alliance GPCV 2000 instrument with online viscometer. The oven temperature is 140 °C. Trichlorobenzene is used as a solvent (ISO 16014).

**The xylene solubles (XS, wt.-%):** Analysis according to the known method: 2.0 g of polymer is dissolved in 250 ml p-xylene at 135°C under agitation. After 30±2 minutes the solution is allowed to cool for 15 minutes at ambient temperature and then allowed to settle for 30 minutes at 25±0.5°C. The solution is filtered and evaporated in nitrogen flow and the residue dried under vacuum at 90 °C until constant weight is reached. $XS % = \left(100\times {m}_{1}\times {v}_{0}\right) / \left({m}_{0}\times {v}_{1}\right) ,$ wherein
m₀ = initial polymer amount (g)
m₁ = weight of residue (g)
v₀ = initial volume (ml)
V₁ = volume of analyzed sample (ml)

**Melting temperature Tm, crystallization temperature Tc, and the degree of crystallinity:** measured with Mettler TA820 differential scanning calorimetry (DSC) on 5-10 mg samples. Both crystallization and melting curves were obtained during 10 °C/min cooling and heating scans between 30 °C and 225 °C. Melting and crystallization temperatures were taken as the peaks of endotherms and exotherms.

Also the melt- and crystallization enthalpy **(Hm and Hc)** were measured by the DSC method according to ISO 11357-3.

**MFR₂:** measured according to ISO 1133 (230°C, 2.16 kg load).

**Comonomer content** is measured with Fourier transform infrared spectroscopy (FTIR) calibrated with ¹³C-NMR. When measuring the ethylene content in polypropylene, a thin film of the sample (thickness about 250 mm) was prepared by hot-pressing. The area of -CH₂- absorption peak (800-650 cm⁻¹) was measured with Perkin Elmer FTIR 1600 spectrometer. The method was calibrated by ethylene content data measured by ¹³C-NMR.

**Stiffness Film TD (transversal direction), Stiffness Film MD (machine direction), Elongation at break TD and Elongation at break MD:** these are determined according to IS0527-3 (cross head speed: 1 mm/min).

**Haze and transparency:** are determined: ASTM D1003-92.

**Intrinsic viscosity:** is measured according to DIN ISO 1628/1, October 1999 (in Decalin at 135 °C).

**Porosity:** is measured according to DIN 66135.

**Surface area:** is measured according to ISO 9277.

**Stepwise Isothermal Segregation Technique (SIST):** The isothermal crystallisation for SIST analysis was performed in a Mettler TA820 DSC on 3±0.5 mg samples at decreasing temperatures between 200°C and 105°C.
(i) The samples were melted at 225 °C for 5 min.,
(ii) then cooled with 80 °C/min to 145 °C
(iii) held for 2 hours at 145 °C,
(iv) then cooled with 80 °C/min to 135 °C
(v) held for 2 hours at 135 °C,
(vi) then cooled with 80 °C/min to 125 °C
(vii) held for 2 hours at 125 °C,
(viii) then cooled with 80 °C/min to 115 °C
(ix) held for 2 hours at 115 °C,
(x) then cooled with 80 °C/min to 105 °C
(xi) held for 2 hours at 105 °C.

After the last step the sample was cooled down to ambient temperature, and the melting curve was obtained by heating the cooled sample at a heating rate of 10°C/min up to 200°C. All measurements were performed in a nitrogen atmosphere. The melt enthalpy is recorded as function of temperature and evaluated through measuring the melt enthalpy of fractions melting within temperature intervals as indicated for example I 1 in the table 3 and figure 4.

The melting curve of the material crystallised this way can be used for calculating the lamella thickness distribution according to Thomson-Gibbs equation (Eq 1.). ${T}_{m} = {T}_{0} ⁢ \left(1-\frac{2 ⁢ σ}{Δ ⁢ {H}_{0} ⋅ L}\right)$
where T₀=457K, ΔH₀ =184x10⁶ J/m³, σ =0,049.6 J/m² and L is the lamella thickness.

### Electrical breakdown strength (EB63%)

It follows standard IEC 60243- part 1 (1988).

The method describes a way to measure the electrical breakdown strength for insulation materials on compression moulded plaques.

### Definition:

${E}_{b} = \frac{{U}_{b}}{d}$
- Eb:: The electrical field strength in the test sample at which breakdown occurs. In homogeneous plaques and films this corresponds to the electrical electrical breakdown strength divided by the thickness of the plaque/film (d), unit: kV/mm.

The electrical breakdown strength is determined at 50 Hz within a high voltage cabinet using metal rods as electrodes as described in IEC60243-1 (4.1.2). The voltage is raised over the film/plaque at 2 kV/s until a breakdown occurs.

### 3. Examples

### Inventive Example 1 (I1)

### Catalyst preparation

The catalyst was prepared as described in example 5 of WO 03/051934, with the Al- and Zr-ratios as given in said example (Al/Zr = 250).

### Catalyst characteristics:

Al- and Zr- content were analyzed via above mentioned method to 36,27 wt.-% Al and 0,42 %-wt. Zr. The average particle diameter (analyzed via Coulter counter) is 20 µm and particle size distribution is shown in Fig. 3.

### Polymerization

A 5 liter stainless steel reactor was used for propylene polymerizations. 1100 g of liquid propylene (Borealis polymerization grade) was fed to reactor. 0.2 ml triethylaluminum (100%, purchased from Crompton) was fed as a scavenger and 15 mmol hydrogen (quality 6.0, supplied by Åga) as chain transfer agent. Reactor temperature was set to 30 °C. 29.1 mg catalyst were flushed into to the reactor with nitrogen overpressure. The reactor was heated up to 70 °C in a period of about 14 minutes. Polymerization was continued for 50 minutes at 70 °C, then propylene was flushed out, 5 mmol hydrogen were fed and the reactor pressure was increased to 20 bars by feeding (gaseous-) propylene. Polymerization continued in gas-phase for 144 minutes, then the reactor was flashed, the polymer was dried and weighted.

Polymer yield was weighted to 901 g, that equals a productivity of 31 kg_{PP}/g_{catalyst}. 1000ppm of a commercial stabilizer Irganox B 215 (FF) (Ciba) have been added to the powder. The powder has been melt compounded with a Prism TSE16 lab kneader at 250rpm at a temperature of 220-230°C.

### Inventive Example 2 (12)

The catalyst was prepared as described in example 5 of WO 03/051934, with the Al- and Zr-ratios as given in said example (Al/Zr = 250).

A 5 liter stainless steel reactor was used for propylene polymerizations. 1100 g of liquid propylene (Borealis polymerization grade) was fed to reactor. 0.2 ml triethylaluminum (100%, purchased from Crompton) was fed as a scavenger and 15 mmol hydrogen (quality 6.0, supplied by Âga) as chain transfer agent. Reactor temperature was set to 30 °C. 17.11 mg catalyst were flushed into to the reactor with nitrogen overpressure. The reactor was heated up to 70 °C in a period of about 14 minutes. Polymerization was continued for 30 minutes at 70 °C, then propylene was flushed out, the reactor pressure was increased to 20 bars by feeding (gaseous-) propylene. Polymerization continued in gas-phase for 135 minutes, then the reactor was flashed, the polymer was dried and weighted.

Polymer yield was weighted to 450 g, that equals a productivity of 17.11 kg_{PP}/g_{catalyst}. 1000ppm of a commercial stabilizer Irganox B 215 (FF) (Ciba) have been added to the powder. The powder has been melt compounded with a Prism TSE16 lab kneader at 250rpm at a temperature of 220-230°C.

### Comparative Example 1 (C1)

A commercial polypropylene homopolymer Borealis has been used.

### Comparative Example 2 (C2)

A commercial polypropylene homopolymer Borealis has been used.

In Table 1, the properties of the polypropylene materials prepared as described above are summarized.

**Table 1: Properties of polypropylene materials**

| | **Unit** | **C1** | **C2** | **I1** | **I2** |
|---|---|---|---|---|---|
| Ash | ppm | 15 | 13 | 85 | - |
| Al | ppm | 1,5 | 1 | 11 | 67 |
| B | ppm | 0 | 0 | 0 | 0 |
| Cl | ppm | 10 | 6 | n.d. | n.d. |
| MFR | g/10' | 2,1 | 2,1 | 2 | 3,8 |
| Mw | g/mol | 412000 | 584000 | 453000 | 367000 |
| Mw/Mn | - | 9,9 | 8,1 | 2,8 | 2,5 |
| XS | wt% | 1,2 | 3,5 | 0,85 | 0,09 |
| mmmm | - | | | 0,95 | 0,95 |
| Tm | °C | 162 | 162 | 150,6 | 150,9 |
| Hm | J/g | 107 | 100 | 99,5 | 96,8 |
| Tc | °C | 115 | 113 | 111,9 | 107,5 |
| Hc | J/g | 101 | 94 | 74,6 | 88,7 |
| g' | - | 1 | 1 | 0,9 | 0,8 |
| SHI | - | 0 | 0 | 0.15 | n/a |
| MBI | - | 0 | 0 | 0.20 | n/a |
| Lamellae Thickness Distribution | - | Broad unimodal | broad unimodal | bimodal | bimodal |
| Chain Architecture | qualitative | linear | linear | branched | Branched |
| SIST Melting <140°C | % | <10% | <10% | >20% | >20% |

In Table 2, the properties of a cast film having a thickness of 80 to 110 µm are summarized. The cast film acts as an exemplary embodiment simulating the properties of a curved cable layer.

**Table 2: Cast film properties**

| | **Unit** | **C1** | **C2** | **I1** | **I2** |
|---|---|---|---|---|---|
| EB63% | kV/mm | 128,9 | 135,2 | 141,5 | 141,4 |
| 90% LOWER CONF: | kV/mm | 124 | 132 | - | 139 |
| 90% UPPER CONF: | kV/mm | 133 | 138 | - | 144 |
| BETA: | none | 17,3 | 26,9 | - | 36,9 |
| Stiffness Film TD | MPa | 960 | 756 | 1011 | 710 |
| Stiffness Film MD | MPa | 954 | 752 | 1059 | 716 |
| Elongation at Break TD | % | 789 | 792 | 700 | 601 |
| Elongation at Break MD | % | 733 | 714 | 691 | 723 |
| Transparency | % | 94 | 94 | 94 | 94 |
| Haze | % | 24,2 | 19,9 | 7,8 | 3,0 |

**Table 3: Results from stepwise isothermal segregation technique (SIST)**

| | | **I1** | **I2** | **C1** | **C2** |
|---|---|---|---|---|---|
| **Peak ID** | **Range [°C]** | **Hₘ [J/g]** | **Hₘ [J/g]** | **Hₘ [J/g]** | **Hₘ [J/g]** |
| 1 | <110 | 6,0 | 4,1 | 0,6 | 1,0 |
| 2 | 110-120 | 3,8 | 3,0 | 1,0 | 1,4 |
| 3 | 120-130 | 4,8 | 5,9 | 2,0 | 2,6 |
| 4 | 130-140 | 11,4 | 19,1 | 3,9 | 4,8 |
| 5 | 140-150 | 27,5 | 35,4 | 10,6 | 12,8 |
| 6 | 150-160 | 29,2 | 37,4 | 25,4 | 32,1 |
| 7 | 160-170 | 16,9 | 2,9 | 50,7 | 56,6 |
| 8 | >170 | 0,1 | 0,0 | 37,5 | 14,3 |

| | | | | | |
|---|---|---|---|---|---|
| **Hₘ** = melting enthalpy | | | | | |

## Claims

1. Cable layer comprising polypropylene, wherein said polypropylene
(a) has a meso pentad concentration higher than 91 %,
(b) is non-crosslinked, and
(c) comprises a crystalline fraction crystallizing in the temperature range of 200 to 105 °C determined by stepwise isothermal segregation technique (SIST), wherein said crystalline fraction comprises a part which during subsequent melting at a melting rate of 10 °C/min melts at or below the temperature T = Tm - 3 °C, wherein Tm is the melting temperature, and said part represents at least 45 wt-% of said crystalline fraction,
and wherein further said polypropylene has been produced in the presence of a symmetric metallocene complex being a transition metal compound of formula (I)
(Cp)₂R₁MX₂ (I)
wherein
M is Zr, Hf or Ti, more preferably Zr
X is independently a monovalent anionic ligand, such as σ-ligand
R is a briding group linking the two Cp ligands
Cp is an organic ligand selected from the group consisting of unsubstituted cyclopentadienyl, unsubstituted indenyl, unsubstituted tetrahydroindenyl, unsubstituted fluorenyl, substituted cyclopentadienyl, substituted indenyl, substituted tetrahydroindenyl, and substituted fluorenyl,
with the proviso that both Cp-ligands are selected from the above stated group and both Cp-ligands are chemically the same, i.e. are identical.

2. Cable layer according to claim 1, wherein said layer and/or the polypropylene of said layer has/have a strain hardening index (SHI@1s⁻¹) of at least 0.15 measured at a deformation rate de/dt of 1.00 s⁻¹ at a temperature of 180 °C, wherein the stain hardening index (SHI) is defined as the slope of the logarithm to the basis 10 of the tensile stress growth function (lg (ηE⁺)) as function of the logarithm to the basis 10 of the Hencky strain (lg (ε)) in the range of the Hencky strains between 1 and 3.

3. Cable layer according to any one of the preceding claims, wherein said layer and/or the polypropylene of said layer has/have xylene solubles below 1.5 wt.-%, preferably below 1.0 wt.-%.

4. Cable layer according to any one of the preceding claims, wherein said layer and/or the polypropylene of said layer has/have xylene solubles in the range of 0.5 to 1.5 wt.-%.

5. Cable layer according to any one of the preceding claims, wherein said layer and/or the polypropylene of said layer comprise(s) at least 90 wt-% of said crystalline fraction.

6. Cable layer according any one of the preceding claims, wherein said layer has a tensile modules of at least 700 MPa measured according to ISO 527-3 at a cross head speed of 1 mm/min.

7. Cable layer according to any one of the preceding claims, wherein said layer and/or the polypropylene of said layer has/have a strain hardening index (SHI@1s⁻¹) in the range of 0.15 to 0.30.

8. Cable layer according to any one of the preceding claims, wherein said layer and/or the polypropylene of said layer has/have a melting point Tm of at least 148 °C.

9. Cable layer according to any one of the preceding claims, wherein said layer and/or the polypropylene of said layer has/have a multi-branching index (MBI) of at least 0.15, wherein the multi-branching index (MBI) is defined as the slope of strain hardening index (SHI) as function of the logarithm to the basis 10 of the Hencky strain rate (lg (dε/dt)), wherein
(a) dε/dt is the deformation rate,
(b) ε is the Hencky strain, and
(c) the strain hardening index (SHI) is measured at a temperature of 180 °C, wherein the strain hardening index (SHI) is defined as the slope of the logarithm to the basis 10 of the tensile stress growth function (Ig (ηE⁺)) as function of the logarithm to the basis 10 of the Hencky strain (Ig (ε)) in the range of the Hencky strains between 1 and 3.

10. Cable layer according to any one of the preceding claims, wherein said layer and/or the polypropylene of said layer has/ave a branching index g' of less than 1.00.

11. Cable layer according to any one of the preceding claims, wherein the polypropylene is multimodal.

12. Cable layer according to any one of the preceding claims 1 to 11, wherein the polypropylene is unimodal.

13. Cable layer according to any one of the preceding claims, wherein the polypropylene has molecular weight distribution (MWD) measured according to ISO 16014 of not more than 8.00.

14. Cable layer according to any one of the preceding claims, wherein the polypropylene has a melt flow rate MFR₂ measured according to ISO 1133 of up to 8 g/10min.

15. Cable layer according to any one of the preceding claims, wherein the polypropylene has a mmmm pentad concentration of higher than 94 % determined by NMR-spectroscopy.

16. Cable layer according to any one of the preceding claims, wherein the polypropylene is a propylene homopolymer.

17. Cable layer according to any one of the preceding claims, wherein said layer has an electrical breakdown strength EB63 % measured according to IEC 60243- part 1 (1988) of at least 135.5 kV/mm. .

18. Cable layer according to any one of the preceding claims, wherein the polypropylene has been produced in the presence of a catalytic system comprising metallocene complex, wherein the catalytic system has a porosity measured according to DIN 66135 of less than 1.40 ml/g.

19. Cable layer according to any one of the preceding claims, wherein the polypropylene has been produced in the presence of a symmetric metallocene complex.

20. A process for the preparation of a cable layer according to any one of the preceding claims 1 to 19, wherein a polypropylene according to any one of the claims 1 to 5, 7 to 19 is formed into a cable layer.

21. The process according to claim 20, wherein the polypropylene is prepared using a catalyst system of low porosity, the catalyst system comprising a symmetric catalyst, wherein the catalyst system has a porosity measured according to DIN 66135 of less than 1.40 ml/g.

22. The process according to claim 21, the catalyst system being a non-silica supported system.

23. The process according to claim 21 or 22, wherein the catalyst system has a porosity below the detection limit of DIN 66135.

24. The process according to any of the preceding claims 21 to 23, wherein the catalyst system has a surface area of less than 25 m²/g, measured according to ISO 9277.

25. The process according to any one of the preceding claims 21 to 24, wherein the symmetric catalyst is a transition metal compound of formula (I)
(Cp)₂R₁MX₂ (I)
wherein
M is Zr, Hf or Ti, more preferably Zr
X is independently a monovalent anionic ligand, such as σ-ligand
R is a briding group linking the two Cp ligands
Cp is an organic ligand selected from the group consisting of unsubstituted cyclopentadienyl, unsubstituted indenyl, unsubstituted tetrahydroindenyl, unsubstituted fluorenyl, substituted cyclopentadienyl, substituted indenyl, substituted tetrahydroindenyl, and substituted fluorenyl,
with the proviso that both Cp-ligands are selected from the above stated group and both Cp-ligands are chemically the same, i.e. are identical.

26. Use of the cable layer according to any one of the preceding claims 1 to 19 in a cable.

27. Cable comprising a conductor and one or more coating layers, wherein at least one of the coating layers is a cable layer according to any one of the preceding claims 1 to 19.

## Patentansprüche

1. Kabelschicht umfassend Polypropylen, worin besagtes Polypropylen
a) eine Mesopentadkonzentration höher als 91 % hat,
b) nicht vernetzt ist, und
c) eine kristalline Fraktion umfasst, die in dem Temperaturbereich von 200 bis 105°C kristallisiert und durch die schrittweise isothermische Abtrennungstechnik (SIAT) bestimmt wird, worin besagte kristalline Fraktion einen Anteil umfasst, welcher während dem anschließenden Schmelzen bei einer Schmelzrate von 10°C/min bei oder unterhalb der Temperatur T = Tm - 3°C schmilzt, worin Tm der Schmelzpunkt ist und besagter Anteil mindestens 45 Gew.-% besagter kristalliner Fraktion darstellt,
und worin weiter besagtes Polypropylen in der Gegenwart eines symmetrischen Metallocenkomplexes hergestellt worden ist, besagter Metallaocenkomplex eine Übergangsmetallverbindung der Formel (I)
(Cp)₂R₁MX₂ (I)
ist, worin
M Zr, Hf oder Ti, mehr bevorzugt Zr, ist
X ein unabhängiger monovalenter anionischer Ligand, wie ein σ-Ligand ist,
R eine die beiden Cp-Liganden verbindende Gruppe ist,
Cp ein organischer Ligand ausgewählt aus der Gruppe bestehend aus unsubstituiertem Cyclopentadienyl, unsubstituierten Indenyl, unsubstituierten Tetrahydroindenyl, unsubstituiertem Fluorenyl, substituierten Cyclopentadienyl, substituierten Indenyl, substituierten Tetrahydroindenyl und substituiertem Fluorenyl ist, mit der Bedingung, dass beide Cp-Liganden aus der oben genannten Gruppe ausgewählt sind, wobei die Cp-Liganden chemisch gleich, d.h. identisch, sind.

2. Kabelschicht nach Anspruch 1, worin besagte Schicht und/oder das Polypropylen der besagten Schicht einen Dehnungsverfestigungsindex (DVI@1sec⁻¹) [strain hardening index (SHI@1sec⁻¹)] von mindestens 0,15 hat/haben, gemessen mit einer Verformungsgeschwindigkeit dε/dt von 1.00 sec⁻¹ bei einer Temperatur von 180°C, worin der Dehnungsverfestigungsindex (DVI@1sec⁻¹) [strain hardening index (SHI@1sec⁻¹)] definiert ist als die Steigung des dekadischen Logarithmus der Zugspannungs-Wachstumsfunktion (lg (η_{ε}⁺)) als Funktion des dekadischen Logarithmus der Hencky Dehnung (lg (ε)) im Bereich der Hencky Dehnung von 1 bis 3.

3. Kabelschicht nach irgendeinem der vorhergehenden Ansprüche, worin besagte Schicht und/oder das Polypropylen der besagten Schicht Xylol-lösliche Anteile unter 1,5 Gew.-%, vorzugsweise unter 1,0 Gew.-%, hat/haben.

4. Kabelschicht nach irgendeinem der vorhergehenden Ansprüche, worin besagte Schicht und/oder das Polypropylen der besagten Schicht 0,5 bis 1,5 Gew.-% Xylol-lösliche Anteile hat/haben.

5. Kabelschicht nach irgendeinem der vorhergehenden Ansprüche, worin besagte Schicht und/oder das Polypropylen der besagten Schicht zumindest 90 Gew.-% besagter kristalliner Fraktion umfasst/umfassen.

6. Kabelschicht nach irgendeinem der vorhergehenden Ansprüche, worin besagte Schicht ein nach ISO 527-3 gemessenes Elastizitätsmodul mit einer transversen Geschwindigkeit von 1 mm/min von mindestens 700 MPa hat.

7. Kabelschicht nach irgendeinem der vorhergehenden Ansprüche, worin besagte Schicht und/oder das Polypropylen der besagten Schicht einen Dehnungsverfestigungsindex (DVI@1 sec⁻¹) [strain hardening index] (SHI@1s⁻¹)] im Bereich von 0,15 bis 0,30 hat/haben.

8. Kabelschicht nach irgendeinem der vorhergehenden Ansprüche, worin besagte Schicht und/oder das Polypropylen der besagten Schicht einen Schmelzpunkt Tm von mindestens 148°C hat/haben.

9. Kabelschicht nach irgendeinem der vorhergehenden Ansprüche, worin besagte Schicht und/oder das Polypropylen der besagten Schicht einen Mehrfach-Verzweigungs-Index (MVI) [multi-branching index (MBI)] von mindestens 0,15 hat/haben, worin der Mehrfach-Verzweigungs-Index (MVI) definiert ist, als die Steigung des Dehnungsverfestigungsindex (DVI) (strain hardening index) (SHI@1s⁻¹)] als Funktion des dekadischen Logarithmus der Hencky Dehnung (lg (dε/dt)), worin
a) dε/dt die Dehnungsgeschwindigkeit ist,
b) ε die Hencky Dehnung ist, und
c) der Dehnungsverfestigungsindex (DVI) [strain hardening index (SHI)] bei einer Temperatur von 180°C gemessen wird, worin der Dehnungsverfestigungsindex DVI [strain hardening index (SHI)] definiert ist als die Steigung des dekadischen Logarithmus der Zugspannungs-Wachstumsfunktion (lg (η_{ε}⁺)), als Funktion des dekadischen Logarithmus der Hencky Dehnung (lg (ε)) im Bereich der Hencky Dehnung von 1 bis 3.

10. Kabelschicht nach irgendeinem der vorhergehenden Ansprüche, worin die Schicht und/oder das Polypropylen der besagten Schicht einen Verzweigungsindex g' von weniger als 1.00 hat/haben.

11. Kabelschicht nach irgendeinem der vorhergehenden Ansprüche, worin das Polypropylen multimodal ist.

12. Kabelschicht nach irgendeinem der Ansprüche 1 bis 10, worin das Polypropylen unimodal ist.

13. Kabelschicht nach irgendeinem der vorhergehenden Ansprüche, worin das Polypropylen eine nach ISO 16014 bestimmte Molekulargewichtsverteilung (MWD) von nicht mehr als 8,00 aufweist.

14. Kabelschicht nach irgendeinem der vorhergehenden Ansprüche, worin das Polypropylen eine nach ISO 1133 bestimmten Schmelzflussrate MFR₂ von bis zu 8 g/10 min aufweist.

15. Kabelschicht nach irgendeinem der vorhergehenden Ansprüche, worin das Polypropylen eine mittels NMR-Spektroskopie bestimmte mmmm Pentadkonzentration von mehr als 94 % aufweist.

16. Kabelschicht nach irgendeinem der vorhergehenden Ansprüche, worin das Polypropylen ein Polypropylenhomopolymer ist.

17. Kabelschicht nach irgendeinem der vorhergehenden Ansprüche, worin besagte Schicht eine nach IEC 60243 Teil 1 (1988) bestimmte Durchschlagsspannung EB 63 % von mindestens 135,5 kV/mm hat.

18. Kabelschicht nach irgendeinem der vorhergehenden Ansprüche, worin das Polypropylen in der Gegenwart eines Katalysatorsystems produziert worden ist, besagtes Katalysatorsystem einen Metallocenkomplex umfasst, worin das Katalysatorsystem eine nach DIN 66135 gemessene Porosität von weniger als 1,40 ml/g aufweist.

19. Kabelschicht nach irgendeinem der vorhergehenden Ansprüche, worin das Polypropylen in Gegenwart eines symetrischen Metallocenkomplexes produziert worden ist.

20. Verfahren zur Herstellung einer Kabelschicht nach irgendeinem der Ansprüche 1 bis 19, worin ein Polypropylen nach irgendeinem der Ansprüche 1 bis 5, 7 bis 19 in eine Kabelschicht geformt wird.

21. Verfahren nach Anspruch 20, worin das Polypropylen unter Verwendung eines Katalysatorsystems mit geringer Porosität hergestellt ist, das Katalysatorsystem einen symmetrischen Katalysator umfasst, worin das Katalysatorsystem eine nach DIN 6135 gemessene Porosität von weniger als 1,40 ml/g hat.

22. Verfahren nach Anspruch 21, worin das Katalysatorsystem ein nicht-silika geträgertes System ist.

23. Verfahren nach Anspruch 21 oder 22, worin das Katalysatorsystem eine Porosität unterhalb des Detektionslimits von DIN 66135 hat.

24. Verfahren nach irgendeinem der Ansprüche 21 bis 23, worin das Katalysatorsystem eine nach ISO 9277 bestimmt Oberfläche von weniger als 25 m²/g aufweist.

25. Verfahren nach irgendeinem der Ansprüche 21 bis 24, worin der symmetrische Katalysator eine Übergangsmetallverbindung der Formel (I)
(Cp)₂R₁MX₂ (I)
ist, worin
M Zr, Hf oder Ti, mehr bevorzugt Zr ist,
X ein unabhängiger monovalenter anionischer Ligand, wie ein σ Ligand, ist,
R eine die beiden Cp-Liganden verbindende Gruppe ist,
Cp ein organischer Ligand ausgewählt aus der Gruppe bestehend aus unsubstituierten Cyclopentadienyl, unsubstituierten Indenyl, unsubstituierten Tetrahydroindenyl, unsubstituierten Fluorenyl, substituiertem Cyclopentadienyl, substituierten Idenyl, substituierten Tetrahydroindenyl und substituiertem Fluorenyl ist,
mit der Bedingung das beide Cp-Liganden aus der oben genannten Gruppe ausgewählt sind, wobei die Cp-Liganden chemisch gleich, d.h. identisch, sind.

26. Verwendung einer Kabelschicht nach irgendeinem der Ansprüche 1 bis 19 in einem Kabel.

27. Kabel umfassend einen Leiter und eine oder mehrere Beschichtungen, worin zumindest eine der Beschichtungen eine Kabelschicht nach irgendeinem der Ansprüche 1 bis 19 ist.

## Revendications

1. Couche de câble comprenant du polypropylène, dans laquelle ledit polypropylène :
(a) a une concentration en mésopentade supérieure à 91 %,
(b) n'est pas réticulé, et
(c) comprend une fraction cristalline qui cristallise dans la plage de températures de 200 à 105 °C déterminée par la technique de ségrégation isotherme progressive (SIST), dans laquelle ladite fraction cristalline comprend une partie qui pendant la fusion ultérieure à une vitesse de fusion de 10 °C / min fond à une température inférieure ou égale à T = Tm - 3 °C, où Tm est la température de fusion, et ladite partie représente au moins 45 % en poids de ladite fraction cristalline,
et dans laquelle en outre ledit polypropylène a été produit en présence d'un complexe de métallocène symétrique qui est un composé d'un métal de transition correspondant à la formule (I)
(Cp)₂R₁MX₂ (I)
où
M est Zr, Hf ou Ti, plus préférablement Zr
X est indépendamment un ligand anionique monovalent, tel que σ-ligand
R est un groupe de liaison reliant les deux ligands Cp
Cp est un ligand organique sélectionné parmi le groupe constitué du cyclopentadiényle non substitué, de l'indényle non substitué, du tétrahydroindényle non substitué, du fluorényle non substitué, du cyclopentadiényle substitué, de l'indényle substitué, du tétrahydroindényle substitué et du fluorényle substitué,
sous réserve que les deux ligands Cp soient sélectionnés dans le groupe susmentionné et que les deux ligands Cp soient chimiquement les mêmes, c'est-à-dire identiques.

2. Couche de câble selon la revendication 1, dans laquelle ladite couche et / ou le polypropylène de ladite couche a / ont un indice d'écrouissage (SHI @ 1s⁻¹) d'au moins 0,15 mesuré à une vitesse de déformation dε/dt de 1,00 s-1 à une température de 180 °C, l'indice d'écrouissage (SHI) étant défini comme la pente du logarithme à la base 10 de la fonction de croissance de la contrainte de traction (lg (η_{E}⁺)) en fonction du logarithme à la base 10 de la contrainte de Hencky (lg (ε)) dans la plage des contraintes de Hencky comprises entre 1 et 3.

3. Couche de câble selon l'une quelconque des revendications précédentes, dans laquelle ladite couche et / ou le polypropylène de ladite couche contient (contiennent) moins de 1,5 % en poids de matières solubles dans le xylène, de préférence moins de 1,0 % en poids.

4. Couche de câble selon l'une quelconque des revendications précédentes, dans laquelle ladite couche et / ou le polypropylène de ladite couche contient (contiennent) des matières solubles dans le xylène dans la plage de 0,5 à 1,5 % en poids.

5. Couche de câble selon l'une quelconque des revendications précédentes, dans laquelle ladite couche et / ou le polypropylène de ladite couche comprend (comprennent) au moins 90 % en poids de ladite fraction cristalline.

6. Couche de câble selon l'une quelconque des revendications précédentes, dans laquelle ladite couche a un module de traction d'au moins 700 MPa mesurés selon la norme ISO 527-3 à une vitesse de traverse de 1 mm / min.

7. Couche de câble selon l'une quelconque des revendications précédentes, dans laquelle ladite couche et / ou le polypropylène de ladite couche a / ont un indice d'écrouissage (SHI @ 1s⁻¹) compris dans la plage de 0,15 à 0,30.

8. Couche de câble selon l'une quelconque des revendications précédentes, dans laquelle ladite couche et / ou le polypropylène de ladite couche a / ont un point de fusion Tm d'au moins 148 °C.

9. Couche de câble selon l'une quelconque des revendications précédentes, dans laquelle ladite couche et / ou le polypropylène de ladite couche a / ont un indice de ramification multiple (MBI) d'au moins 0,15, dans laquelle l'indice de ramification multiple (MBI) est défini comme la pente de l'indice d'écrouissage (SHI) en fonction du logarithme à la base 10 de la vitesse de déformation de Hencky (lg (dε / dt)), où
(a) dε / dt est la vitesse de déformation,
(b) ε est la contrainte de Hencky, et
(c) l'indice d'écrouissage (SHI) est mesuré à une température de 180 °C, l'indice d'écrouissage (SHI) étant défini comme la pente du logarithme à la base 10 de la fonction de croissance de la contrainte de traction (lg (η_{E}⁺)) en fonction du logarithme à la base 10 de la contrainte de Hencky (lg (ε)) dans la plage des contraintes de Hencky comprises entre 1 et 3.

10. Couche de câble selon l'une quelconque des revendications précédentes, dans laquelle ladite couche et / ou le polypropylène de ladite couche a / ont un indice de ramification g' inférieur à 1,00.

11. Couche de câble selon l'une quelconque des revendications précédentes, dans laquelle le polypropylène est multimodal.

12. Couche de câble selon l'une quelconque des revendications 1 à 11 précédentes, dans laquelle le polypropylène est unimodal.

13. Couche de câble selon l'une quelconque des revendications précédentes, dans laquelle le polypropylène a une répartition du poids moléculaire mesurée selon la norme ISO 16014 inférieure ou égale à 8,00.

14. Couche de câble selon l'une quelconque des revendications précédentes, dans laquelle le polypropylène a un indice de fluidité MFR₂ mesuré selon la norme ISO 1133 de 8 g / 10 min. maximum.

15. Couche de câble selon l'une quelconque des revendications précédentes, dans laquelle le polypropylène a une concentration en pentade mmmm supérieure à 94 % déterminée par spectroscopie RMN.

16. Couche de câble selon l'une quelconque des revendications précédentes, dans laquelle le polypropylène est un homopolymère de propylène.

17. Couche de câble selon l'une quelconque des revendications précédentes, dans laquelle ladite couche a une résistance aux décharges électriques EB 63 % mesurée selon la norme IEC 60243 - 1^{ère} partie (1988) d'au moins 135,5 kV / mm.

18. Couche de câble selon l'une quelconque des revendications précédentes, dans laquelle le polypropylène a été produit en présence d'un système catalytique comprenant un complexe de métallocène, le système catalytique ayant une porosité mesurée selon la norme DIN 66135 inférieure à 1,40 ml / g.

19. Couche de câble selon l'une quelconque des revendications précédentes, dans laquelle le polypropylène a été produit en présence d'un complexe de métallocène symétrique.

20. Procédé de préparation d'une couche de câble selon l'une quelconque des revendications 1 à 19 précédentes, dans lequel un polypropylène selon l'une quelconque des revendications 1 à 5 et 7 à 19 est façonné de manière à en faire une couche de câble.

21. Procédé selon la revendication 20, dans lequel le polypropylène est préparé à l'aide d'un système de catalyseur de faible porosité, le système de catalyseur comprenant un catalyseur symétrique et ayant une porosité mesurée selon la norme DIN 66135 inférieure à 1,40 ml / g.

22. Procédé selon la revendication 21, le système de catalyseur étant un système non supporté par de la silice.

23. Procédé selon la revendication 21 ou 22, dans lequel le système de catalyseur a une porosité inférieure au seuil de détection défini par la norme DIN 66135.

24. Procédé selon l'une quelconque des revendications 21 à 23 précédentes, dans lequel le système de catalyseur a une superficie inférieure à 25 m² / g, mesurée selon la norme ISO 9277.

25. Procédé selon l'une quelconque des revendications 21 à 24 précédentes, dans lequel le catalyseur symétrique est un composé d'un métal de transition correspondant à la formule (I)
(Cp)₂R₁MX₂ (I)
où
M est Zr, Hf ou Ti, plus préférablement Zr
X est indépendamment un ligand anionique monovalent, tel que σ-ligand
R est un groupe de liaison reliant les deux ligands Cp
Cp est un ligand organique sélectionné parmi le groupe constitué du cyclopentadiényle non substitué, de l'indényle non substitué, du tétrahydroindényle non substitué, du fluorényle non substitué, du cyclopentadiényle substitué, de l'indényle substitué, du tétrahydroindényle substitué et du fluorényle substitué,
sous réserve que les deux ligands Cp soient sélectionnés dans le groupe susmentionné et que les deux ligands Cp soient chimiquement les mêmes, c'est-à-dire identiques.

26. Utilisation de la couche de câble selon l'une quelconque des revendications 1 à 19 précédentes dans un câble.

27. Câble comprenant un conducteur et une ou plusieurs couches de revêtement, dans lequel au moins une des couches de revêtement est une couche de câble selon l'une quelconque des revendications 1 à 19 précédentes.
